

F. LAIST.

PROCESS OF ROASTING ORES.

APPLICATION FILED NOV. 22, 1913.

1,114,372.

Patented Oct. 20, 1914.



WITNESSES:

Harry A. Reiner  
Jos. Amichay

INVENTOR.  
Frederick Laist.

BY  
Emil Starey  
ATTORNEY.

# UNITED STATES PATENT OFFICE.

FREDERICK LAIST, OF ANACONDA, MONTANA.

## PROCESS OF ROASTING ORES.

1,114,372.

Specification of Letters Patent.

Patented Oct. 20, 1914.

Application filed November 22, 1913. Serial No. 802,480.

To all whom it may concern:

Be it known that I, FREDERICK LAIST, a citizen of the United States, residing at Anaconda, in the county of Deerlodge and 5 State of Montana, have invented certain new and useful Improvements in Processes of Roasting Ores, of which the following is a full, clear, and exact description, reference being had to the accompanying drawings, 10 forming a part hereof.

My invention has relation to improvements in processes of roasting ores; and it consists in the novel features more fully 15 set forth in the specification and pointed out in the claims.

In the drawings, the figure is a combined elevation and middle vertical section of a furnace adapted to carry out my process, the section being taken through one of the fire-boxes.

The basic principle involved in the present process is disclosed in my United States patent on roasting furnace, dated August 19, 1913, Number 1,070,490, said furnace being 20 one of the forms designed for carrying out the process.

The invention relates to processes of treating ores, the particular treatment depending on the character and composition of the ore 30 (or other material).

The process is specially adapted for roasting copper sulfid ores, and for roasting and chloridizing such ores when containing silver, and is eminently desirable for treating low 35 grade ores to bring their metal constituents into a form suitable for leaching and final recovery by precipitation or otherwise.

To the principle involved in the process, the saving of a large percentage of fuel is 40 mainly due, one of the objects sought by my invention being to minimize the consumption of fuel employed for firing the charge to be treated.

A further object of my invention is to 45 avoid undue volatilization of metallic chlorides especially in the roasting and chloridizing of copper ores, this being a decided advantage of my process; and it results from the fact that the chloridation of the hot 50 roasted calcine is carried on without the application thereto either of extraneous heat, or without dependence on heat of combustion within the mass, and under conditions where the reactions involving the

chloridation are not affected by the cooling 55 influences of the atmosphere.

To obtain a clear understanding of the improved process, it will be convenient to describe a form of furnace in which the invention may be practised to advantage. 60 The furnace shown and described in my patent aforesaid, altered in one or two minor details, is eminently adapted for carrying on my process, although it is not to be considered as the only apparatus or furnace 65 available for my purpose. However, inasmuch as the furnace referred to has in practice been identified with the basic principle of my invention, it will be convenient to describe my process in connection with 70 said furnace, only so much of the description of the latter being herein entered into, as will suffice to make intelligible the details of the process.

The invention may be described in detail 75 as follows:

Referring to the drawing, F, represents the furnace (extending partly above and partly below the floor-line L), and a, b, c, d, e, f, the several superposed hearths in 80 which the material is treated (the present being a six-hearth multiple-hearth furnace), the material delivered from the feed-hopper H dropping from the upper hearths successively through the several hearths until 85 it is delivered into the discharge hopper C, the hearths being provided with the central and marginal openings or drop-holes o, o', for the passage of the material. Passing centrally through the hearths is the rotatable hollow rabble-shaft 1 from which radiate the series of hollow rabble or stirrer arms 2 extending into the several hearths and carrying rakes 3, by which the material is 90 successively fed from one hearth to the hearth immediately beneath it, the shaft and arms being provided with air or water-circulating cooling pipes P, P', as fully understood in the art.

The present is a direct-fired furnace being 100 provided with two diametrically opposite fire-boxes B, burning coal (though coal-dust, oil, or gas may be substituted), each fire-box having a shaking grate G, an ash launder A, and a checker-work arch W, and discharging 105 its gases and combustion products into the hearth e or hearth number three counting from the top. This hearth is considerably

deeper than any of the remaining hearths there being left a clearance of from ten to twelve inches between the upper surface of the rabble-arms in said hearth and the roof 5 of the hearth, the gases from the fire-boxes discharging into said hearth through the openings  $\sigma$  which are located above the rabble arms and contiguous to the outer edge of said roof. As seen in the drawing, the marginal drop holes  $\sigma'$  of the second hearth (b) 10 (always counting from the top) discharge the material onto the floor of the third hearth c. In hearth c the roasting ore is moving away from the circumference toward the center drop hole  $\sigma$ . The ore is likewise moving away from the fire-boxes, this being an important feature of my invention for the following reason:—In any direct-fired furnace used for roasting copper 15 ore for leaching purposes, it is very important to avoid overheating any of the ore since to do so causes a portion of the copper contents to become insoluble in the leaching solution, owing to the formation of ferrite copper. The temperature on the 20 second floor or hearth b is by measurement approximately 540 degrees Fahr. about two feet radially from the point where the ore drops onto the third floor (c). Before the 25 formation of "insoluble copper" (ferrite copper) becomes serious a temperature of at least 1100 degrees Fahr. must be exceeded, so that the quantity of insoluble copper on this floor (b) is negligible and it makes no 30 difference what the relative movement of the ore and flame thereover may be. On the third floor (c) however, conditions are different. Here we have a temperature of 1280 degrees Fahr. about two feet from the 35 furnace walls and about midway between the drop-holes (from hearth b) and the gas discharge or fire-box openings  $\sigma$ , the temperature being even higher closer to the said openings. The ore dropping from the 40 second floor (b) has a temperature of about 500 degrees Fahr.; and were it permitted to move toward this region or zone of high temperature, the tendency would be for portions of the ore to become overheated and 45 rendered insoluble as above pointed out. This overheating will obviously be much reduced by having the comparatively cool ore entering said heated region or zone, moved continually toward a region of less 50 heat or lower temperature, that is to say, toward the center of the hearth. Accordingly, in a multiple-hearth furnace, roasting ore for leaching by direct firing, it is essential 55 that the direct-fired hearth shall be one in which the ore is moved toward the center or away from the zone of high temperature prevailing at the point of discharge of the gases from the fire-box into the hearth. In 60 my present construction therefore, the fire-

box is allowed to discharge into the third 65 hearth c in which the rakes move the ore from the circumference toward the center. It is also important, in order to minimize the formation of insoluble or ferrite copper, and to prevent the destruction and deterioration of the rabble arms and rakes in 70 this hearth (c) that the openings  $\sigma$  from the fire boxes shall be immediately under the roof of the third hearth, and that this roof shall be so high above the rabble arms 75 that the flame will clear the arms and play between the roof and said arms. It is for this reason that a clearance of from ten to twelve inches is left between the upper surface of the rabble arms and the roof of the 80 third hearth, the rabble arms being thus brought out of range of the gases from the openings  $\sigma$ .

It is stated in my patent aforesaid that there are generally speaking "two types of 85 roasts made use of for rendering soluble in dilute acids the copper contents of sulfid ores, to-wit:—(1,) an oxidizing or sulfating roast, and (2,) a chloridizing roast." In this classification of the types of roasts the 90 term "oxidizing" must be considered in its generic sense, because whether the metal is converted into  $\text{CuO}$ , or  $\text{CuSO}_4$ , it must be oxidized, that is to say, the  $\text{Cu}_2\text{S}$  is first converted into  $\text{CuO}$  and  $\text{SO}_2$ , any  $\text{SO}_3$  which 95 may form converting the  $\text{CuO}$  to  $\text{CuSO}_4$ , and the result is a mixture of  $\text{CuO}$  and  $\text{CuSO}_4$ , the sulfating process being likewise an "oxidizing" one, speaking generically. Specifically however, these types may be 100 considered as three distinct types, to-wit:—(a) the oxidizing roast pure and simple which contemplates the conversion of the metal to the oxid; (b) the sulfating roast which contemplates the formation of the 105 sulfate of the metal; and (c) the chloridizing roast by which metallic oxides and sulfates (together with undecomposed sulfids, such as the sulfid of silver where silver is present) are converted into the chlorids 110 of the metals.

My process contemplates the practice of either the first two types, or it may combine all three, depending on whether silver is absent or present in the ore. If no silver is 115 present, the ore charge is subjected merely to an oxidizing and sulfating roast; if silver is present then the charge is subjected to a combination of oxidizing, sulfating and chloridizing roasts. The ore is oxidized on 120 the three upper hearths or floors a, b, c, sulfated on the three lower floors d, e, f, or sulfated and chloridized on said lower floors depending on the composition of the ore, the temperature of the charge being 125 raised sufficiently high on the oxidizing floors to permit of a subsequent rapid sulfating, or combined sulfating and chloridiz-

ing action on the lower floors. The furnace walls of the three lower floors are insulated against heat loss by radiation by a layer of asbestos 19 or its equivalent, or by making 5 the walls sufficiently thick to prevent loss of heat, or by means of an air space, the bottom floor being likewise properly insulated. The insulation referred to is important since the lower floors (d, e, f) in which 10 the sulfating, or the sulfating and chloridation are taking place, are heated solely by the heat of the calcine or roasted material discharged from the upper or oxidizing hearths or floors, and which works 15 down through said floors.

Assuming that the ore treated is a copper sulfid with more or less iron as an impurity, but carrying no silver, the product of the oxidizing roast from the hearths a, b, c, is 20 mainly CuO, FeO, (very little sulfating taking place on these floors so that the amount of CuSO<sub>4</sub>, and FeSO<sub>4</sub> need not be considered). On the three lower floors 25 d, e, f, any undecomposed sulfids will be converted into sulfates, the SO<sub>2</sub> in the presence of oxygen (air entering these floors through an opening E in the wall of the bottom hearth f) being converted into SO<sub>3</sub>, which, combining with CuO, converts the 30 latter into CuSO<sub>4</sub>, the iron (and alumina if any) being likewise sulfated. This sulfating roast however, is effected without any direct fire from without, (and without material dependence of the heat of oxidation 35 of the sulfur still remaining in the charge while traversing the lower hearths) but depends for its consummation on the heat conserved in the calcines as they drop from the upper oxidizing (a, b, c) to the lower sulfating hearths (d, e, f), and while traversing said lower hearths.

Again, assuming that the ore treated is a copper sulfid carrying silver, the product of the oxidizing roast from the hearths a, b, c, 45 is probably a mixture of CuO, FeO, Ag, Ag<sub>2</sub>S, with small quantities of Cu<sub>2</sub>S, CuSO<sub>4</sub>, Ag<sub>2</sub>SO<sub>4</sub> and FeSO<sub>4</sub>. In this case there takes place on the lower hearths (d, e, f) a sulfating reaction similar to that above described, and concurrently therewith a chloridizing reaction, common salt (NaCl) being added to chloridize the silver. The salt is fed to the fourth floor (d) in proper quantities, either through the doors D or by 50 means of any suitable form of automatic feeder discharging the salt onto the hearth at a convenient point, and well understood in the art. The temperature of the floor (d) in which the salt is introduced is any 55 where from 850 to 1000 degrees Fahrenheit, this being sufficient to permit the salt (which is introduced cold) to react with the metal constituents contained in the hot calcines, the reactions continuing throughout the several 60

chloridizing hearths. The salt chloridizes 65 all the silver present and that portion of the copper (CuSO<sub>4</sub>) which may have escaped conversion into oxid on the upper floors, although it is quite probable that a small portion of the copper oxid will likewise be converted into chlorid, the chlorid of iron which is likewise formed being broken up into the oxid by the heat and oxygen present. The reactions identified with the chloridizing step of the process are probably as follows:— 75



Any unconverted copper sulfate, and copper oxid is discharged from the furnace with the silver chlorid and copper chlorid, and with any iron oxid present in the chloridized charge. The final product or calcine is cooled in any suitable ore cooler known to 85 the art, and is subsequently leached, the leaching solution employed being water containing from three to fifteen per cent. by weight of sulfuric acid and from four to fifteen per cent. by weight of common salt, 90 such solution readily dissolving the several components of the calcine referred to (the gangue and sand of course being insoluble). The dissolved metallic salts may be subsequently recovered by precipitation or 95 by any other method known to the art.

In all chloridizing-roasting, a certain percentage of the copper (usually as chlorid) volatilizes; and while under my process this percentage is reduced to a minimum, yet 105 provision is herein made to save and condense these copper fumes (and any chlorin and SO<sub>3</sub>) by leading the furnace gases (from the pipes 25, 26 or otherwise) to a suitable absorption tower or Cottrell electric 110 precipitation apparatus, or both (not shown), a corresponding quantity of air being admitted to the chloridizing and sulfating hearths (d, e, f) through an opening E in the bottom hearth (f), the oxygen of 115 the air so admitted facilitating the chloridizing (and sulfating) reaction in said hearths (d, e, f) and the air current assisting in carrying off any volatile chlorids.

By my process the ore is brought rapidly 120 to a roasting temperature, the oxidizing roast eliminating a considerable proportion of the sulfur in the form of SO<sub>2</sub>, small portions in this roast entering in combination with portions of the metallic bases forming 125 sulfates. The bulk of the metal (copper, where copper is roasted) is however converted into the oxid. The roasted ore or hot

calcine without loss of heat, and fully insulated from the cooling influences of the atmosphere by the walls of the lower insulated section of the furnace, drops, or is conducted into, the chloridizing or sulfating hearths (d, e, f) where the chloridizing or sulfating reaction completes itself in a manner similar to that of the contents of a fireless cooker, that is to say, without accession or application, of extraneous heat. It may be stated in passing that the feed to the furnace contains from 2.5 to 3 per cent. of sulfur and still contains about one per cent. of sulfur when it drops from the third (c) to the fourth (d) hearth or floor. The finished calcine (that is to say, the product as it leaves the chloridizing or sulfating hearths) contains about five-tenths of one per cent. of sulfur, of which one-tenth of one per cent. is in the form of undecomposed sulfids and four-tenths of one per cent. in the form of sulfates. Of the one per cent. of sulfur present in the calcine as it drops from the third to the fourth hearth about nine-tenths is in the form of undecomposed sulfids, and one-tenth in the form of sulfates. It follows therefore that the quantity of sulfid decomposed or oxidized in the chloridizing or sulfating hearths is about eight-tenths of one per cent. That is to say, of the nine-tenths per cent. of sulfids dropping from the third to the fourth hearth, three-tenths have been converted into sulfates, which three-tenths added to the one-tenth dropping into the chloridizing or sulfating hearths, makes up the final four-tenths of sulfates in the finished calcine. One-tenth of the nine-tenths per cent. of sulfid dropping from the third to the fourth hearth remains undecomposed in the finished calcine, the sulfur of the remaining five-tenths of the nine-tenths sulfid oxidizing or being converted into  $\text{SO}_2$  or  $\text{SO}_3$  fumes (which are abstracted with any volatile copper chlorid fumes and drawn into the absorption tower). The heat of oxidation from this small quantity of sulfur is negligible as compared with the great amount of heat developed in the oxidizing hearths, and with which the calcines are charged as they enter the chloridizing hearths, this heat being that on which dependence is placed to bring about the necessary reaction between the salt and the metal constituents of the calcines.

It will thus be seen that no attempt is made herein to rely on the undecomposed sulfid content of the ore for the generation of heat (by oxidation) in the chloridizing or sulfating hearths, the object sought being to decompose to the extent indicated, the sulfids in the oxidizing hearths, the sulfur in the main passing off as  $\text{SO}_2$ . Any sulfates which are formed, (and a portion of the oxids ( $\text{CuO}$ ) present) freely react

with the salt ( $\text{NaCl}$ ) added in the second stage of the process, the nascent chlorin attacking the metals and converting the same into chlorids, as per reactions given above. The decomposition of the sulfids in the oxidizing hearths (a, b, c) is brought about by the high temperature of the fire gases from the fire-boxes B, operating in conjunction with the hot air and gases discharged into said hearths from the sulfating hearths d, e, f, (through the drop hole o between the hearths c and d), said air and gases passing over and between the particles of the ore in its travel through the several hearths, whereby the gases reach every portion of the ore. The decomposition of the sulfids by the oxidizing roast leaves but a small percentage of undecomposed sulfid to contend with in the chloridizing and sulfating hearths (the major portion in said hearths being probably silver sulfid). Thus the sulfur element as a fuel and heat generator is practically eliminated in the chloridizing hearths, dependence being placed substantially entirely on the heat conserved in the roasted calcines discharged from the oxidizing hearths (a, b, c), to effect the necessary reaction between the salt (added to the calcines in the chloridizing or sulfating hearths) and the metal constituents of the calcines. Practically no heat (a negligible quantity) is generated in the chloridizing or sulfating hearths (unless it be that due to the chemical reactions above referred to) from the combustion of sulfur; and no conserved heat is dissipated, because the walls of the furnace are effectively insulated. The result is a perfect chloridation with a minimum volatilization of copper chlorid.

The process is adapted for treatment of any grade of ore, but specially low grade ores where it is desirable to bring their metal content into a soluble form for precipitation or other form of recovery.

The process is not to be understood as restricted to the treatment of "ores" any other material adapted to be roasted, calcined, oxidized, and subsequently sulfated or chloridized being contemplated by the invention.

It may be stated in passing that the insulated walls of the lower section of the furnace while serving to conserve the heat in the mass or calcine discharged from the oxidizing into the chloridizing or sulfating hearths, preventing as they do a dissipation of the heat, at the same time protect the calcines from the cooling influence of the atmosphere, the object sought being to make the insulation as complete as possible.

Features of furnace construction illustrated but not alluded to are fully described in my patent aforesaid, and there is no occa-

sion to describe them in the present connection.

The fuel employed in my process (in the fire-boxes B, B) being restricted in its application to the oxidizing hearths (a, b, c), it follows that less fuel is required than would be the case were the bottom hearths (d, e, f) also fired. The process is therefore exceedingly economical of fuel. The bottom hearths it will be seen, serve both as sulfating and chloridizing hearths; sulfating alone where no salt is used, and sulfating and chloridizing where salt enters into the reaction.

Having described my invention, what I claim is:—

1. In the treatment of ores and other material, the process of subjecting a charge of the ore while traversing a treatment chamber to the action of hot reaction-supporting gases, introducing said gases in a direction conforming to the general direction of movement of the ore in said chamber to prevent overheating of the charge, removing the resulting hot calcines from the influence of the said gases completing the treatment of the calcines thus removed without further application of heat, and conducting the gases from the final treatment, to the charge traversing the treatment chamber aforesaid.

2. In the treatment of ores and other material, the process of subjecting a charge of the ore while traversing a treatment chamber to the action of hot reaction-supporting gases, removing the resulting hot calcines from the influence of said gases, completing the treatment of the calcines thus removed without further application of heat, and conducting the gases from the final treatment, to the charge traversing the treatment chamber aforesaid.

3. In the treatment of ores and other material, the process of subjecting a charge of the ore while traversing a treatment chamber to the action of hot reaction-supporting gases, removing the hot calcines from the influence of said gases, conducting said calcines in a heat-insulated chamber, completing the treatment of the calcines in said heat-insulated chamber without further application of heat, and conducting the gases from the final treatment, to the charge traversing the treatment chamber.

4. In the treatment of ores and other material, the process of subjecting the ore while traversing a treatment chamber to the direct fire of furnace gases within said chamber, moving said charge from a zone of high, to a region of comparatively low temperature, while in contact with said gases, removing the hot calcines from said region of low temperature to a heat-insulated chamber, completing the reaction within the mass, in said chamber without further application of heat, and conducting the hot calcines to the one in treatment chamber.

5. In the treatment of ores, the process of subjecting the ore while traversing a treatment chamber to the direct fire of furnace gases within said chamber, stirring said charge in the chamber and moving the same from a zone of high, to a region of comparatively low temperature while in contact with said gases, removing the hot calcines from said region of low temperature to a heat-insulated chamber, mixing with the calcines a quantity of salt and stirring the mixture in said insulated chamber in the presence of oxygen without further application of heat, and conducting the hot air and gases of the final reaction to the ore in the treatment chamber.

6. In the treatment of ores, the process of subjecting a charge of the ore traversing a series of intercommunicating treatment chambers to the action of hot reaction gases circulating through said chambers, and initially directed into the chamber last traversed by the ore, moving the ore in said last mentioned chamber from a zone of high, to a region of comparatively low temperature while in contact with the gases, removing the calcines from the region of low temperature and conducting the same to a heat-insulated chamber, stirring the calcines in said chamber without further application of heat, to complete the reaction, and conducting the gases of the completed reaction into the chamber into which the first hot reaction gases are initially directed.

7. In an oxidizing, sulfating, and chloridizing of ores, the process of feeding the ore successively through a series of intercommunicating treatment chambers, directing hot reaction-gases into the last chamber of said series and causing the gases to circulate through the several chambers, moving the charge immediately entered by the reaction gases from a zone of high to a region of comparatively low temperature, removing the hot calcines from said region of low temperature, feeding the same through a succession of heat-insulated treatment chambers in the presence of salt and oxygen, stirring the mixture while traversing said insulated chambers, whereby the reaction completes itself without further application of heat, and conducting the gases from said heat insulated chambers to the charge traversing the first treatment chambers.

8. In the treatment of ores and other material, the process of subjecting a charge of the ore while traversing a treatment chamber to the action of hot reaction gases for oxidizing the charge, removing the hot calcines from the influence of said gases, conducting the same into a heat-insulated

chamber, stirring the calcines in said chamber in the presence of oxygen, whereby the treatment is completed without further application of heat, and conducting the hot air and gases of the final reaction from said heat-insulated chamber into the first mentioned treatment chamber.

In testimony whereof I affix my signature, in presence of two witnesses.

FREDERICK LAIST.

Witnesses:

ALBERT E. WIGGIN,  
WARREN JENNEY.